

## UNITED STATES PATENT OFFICE

2,241,575

METHOD OF MAKING CAST IRON AND  
ADDITION MATERIAL THEREFOR

Thomas E. Barlow, Columbus, Ohio, assignor to  
Battelle Memorial Institute, Columbus, Ohio, a  
corporation of Ohio

No Drawing. Application March 24, 1939,  
Serial No. 263,958

2 Claims. (Cl. 75—130)

This invention relates to a method of making cast iron and addition material therefor. It has to do particularly with the treatment of the cast iron when it is in a molten state.

In the prior art, it has been known for some time that cast iron melted under some conditions and cast into various sections and shapes may exhibit a fine, lacy and frequently dendritic graphite formation. These irons are commonly referred to as "dendritic cast irons," "modified cast irons" or "under cooled cast irons." This lacy type of graphite is frequently associated with patches of ferrite, commonly referred to as "snow-balls" or "primary ferrite" to differentiate from the ferrite which is normally found in certain compositions. Although "modified" or "dendritic" cast iron is said to have certain uses such as in the manufacture of heat resistant castings, it is found to exhibit lower tensile and transverse strength, lower deflection, lower resilience, decreased wear resistance and greater tendency to chill than the so-called normal irons. For these reasons the "modified" structure is deemed to be unsuited to the majority of the uses of cast iron.

There are a number of alloys on the market today which will, to some extent, eliminate the tendency of gray iron to modify. One of the most common of these and the one on which the most work has been done is ferrosilicon. Unfortunately, however, the use of ferrosilicon is accompanied by a tendency towards shrinkage, blow-holes and porosity. To obtain maximum effects from ferrosilicon, it is frequently necessary to add as much as 1.50 per cent silicon to the ladle. When adding more than 1.00 per cent silicon the tendency to form blow-holes and shrinks becomes increasingly pronounced. With 1.5 per cent silicon or more added to the ladle, it is almost impossible to cast completely sound test bars in green sand. The amount of ferrosilicon which may be used without danger of promoting porosity and low strength is frequently insufficient to offset the tendency of the iron to modify. This is especially true of superheated irons.

Various other alloys have been used as ladle additions for the purpose of preventing modification of cast iron with some success. An alloy of titanium, aluminum, silicon and iron has been somewhat successful but the indications are that it is unduly concentrated to enable it to obtain

the best results. The addition of more than 3 ounces of this alloy per hundred pounds of iron seems to be actually harmful.

Calcium silicide has been used as a ladle addition to prevent the modification of the cast iron. However, the fumes ensuing from its use are rather objectionable and there is room for improvement in the results attainable therewith.

Silicon carbide is somewhat successful for the purpose in question. However, the increase in carbon and silicon resulting from its use tends to offset the beneficial effects thereof.

It has been found that the use of pure aluminum in the foundry for the purpose of preventing modification of cast iron is not advantageous. Apparently, the aluminum accumulates during melting and causes pin-holes and blow-holes. Also, the aluminum is so potent as a ladle addition that the slightest excess causes these same casting defects. It is claimed that if the ladle addition alloy contains twice as much silicon as aluminum, the two elements flux off as a low melting point slag and that this prevents the aluminum content from building up to the danger point. However, even the combination of silicon and aluminum in the proportions indicated for the production of an alloy to be used in preventing modification of the cast iron leaves something to be desired.

One of the objects of this invention is to provide a method and an alloy for use therein which will relieve the above-mentioned modified structural deficiencies of the graphite in the iron.

Another object of this invention is to produce an alloy for the purpose indicated which will be intrinsically beneficial to the physical and mechanical properties of the cast iron, instead of being detrimental or neutral in its effect upon such physical and mechanical properties.

This invention consists in the conception and verification of the fact that a method of making cast iron can be greatly improved by introducing into the cast iron, while it is in molten form, a copper base alloy which preferably contains aluminum and silicon and which may also contain manganese. It has been found that the introduction of such an alloy into the molten cast iron is far superior to the effects of any of its components when they are added separately. The effect of such a single alloy as an addition material for the cast iron is also superior to the com-

bined effects of all its components when they are added as ferrosilicon, ferromanganese, copper shot and aluminum wire, for example. The superiority is apparently at least partly due to (1) the superior distribution of the individual elements when added as a single alloy and (2) the low melting point of the alloy which is approximately 1500° F. When my alloy is added to cast iron, it not only relieves or eliminates the above-mentioned "modified" structural conditions of the graphite in the iron but it also introduces an alloying element or elements intrinsically beneficial rather than detrimental or neutral to the improvement of the physical and mechanical properties of the cast iron.

Copper was decided upon as a base for the alloy for three reasons. In the first place, tests have shown that copper in itself has a tendency to relieve the "modified" condition referred to above. Secondly, copper imparts definite benefits to cast iron, especially in regard to increasing density, decreasing chill, decreasing section sensitivity, increasing machinability and increasing strength and toughness. Also, large additions of copper do not tend to cause foundry defects such as blow-holes, pin-holes, shrinks, etc. In the third place, copper is a low priced metal and is readily available.

Aluminum was chosen as the chief "deoxidizing" element. It was felt, and later proved, that no harmful effects would result from the use of aluminum when diluted with a large amount of other elements such as copper. Also, when diluted with copper, no difficulty was had in getting uniform distribution of the aluminum in the molten cast iron bath. Another point of some consequence is the fact that a small amount of aluminum is said to produce better distribution of copper in cast iron.

One undesirable feature of aluminum additions to cast iron is the fact that a finely divided oxide is formed which is frequently difficult to separate from the molten cast iron. These oxide particles frequently cause foundry defects. For this reason, silicon is added to the alloy and, as indicated, manganese may also be added. When the correct ratio of silicon or of silicon and the manganese to aluminum is present, a low melting point slag is formed which readily separates from the molten metal. In addition, both silicon and manganese have a beneficial effect in regard to elimination of "dendritic" graphite. In no case is it necessary to maintain the silicon and manganese contents of the alloy so high as to introduce any weakening effect into the resulting cast iron. In fact, the addition of manganese, especially in the presence of copper, is known to strengthen rather than weaken cast iron.

The range of composition which is best suited for the aluminum, silicon, copper alloys is as follows:

|          | Percent  |
|----------|----------|
| Aluminum | 1 to 10  |
| Silicon  | 6 to 25  |
| Copper   | 50 to 93 |

If manganese is to be used in the alloy, it may be present in percentages ranging up to 25%. However, in this case the quantity of silicon may be reduced to between 10% and 15%.

In practice, it is desirable that the silicon and manganese be introduced as ferrosilicon or ferromanganese. In this event, the amount of iron present may be varied over a wide range, due to the fact that it is merely a diluent. Thus, the

iron may be present in percentages up to 30%. However, dilution of this alloy with iron would necessitate a larger addition of the alloy to the molten cast iron and is therefore not desirable.

5 The cost of producing the alloy can be materially lowered by introducing the silicon and manganese as ferrosilicon and ferromanganese thereby introducing some iron. Also, iron is a common impurity in many of the materials of manufacture.

10 However, the best results can be obtained by maintaining the iron content below 10%.

It is preferable that the percentages of the various elements comprising either the aluminum, silicon, copper alloy or the aluminum, sili-

15 con, manganese, copper alloy should be such that

1% of the alloy added to the molten iron will be sufficient to offset any ordinary tendency of the iron to modify. It is desirable to have the alloy sufficiently dilute to require 1% so as to take

20 advantage of the apparent mass action effect involved and also to ensure better distribution of the more powerfully deoxidizing elements present such as aluminum and silicon. However, it is not advisable to have the alloy so dilute that more

25 than 1% is required because of the reduction of metal temperature effected by large ladle additions.

Due to the low melting point of the alloy, 1%

30 can be added with no difficulty and still permit the addition of ferrochromium, ferromolybdenum, ferrovanadium, nickel, copper and other alloys which are frequently added for special purposes.

In unusual cases, where a large degree of modi-

35 fication is encountered or where it is desirable to add more copper for special purposes, up to 2% of the alloy can be added without excessive chilling of fairly hot molten iron. It has been found that this alloy unlike other "deoxidizers" such as silicon and aluminum, is not detrimental when

40 added in excess of the recommended amount.

Aluminum contents of less than 1% would not be sufficient for efficient "deoxidation". Over

45 10% aluminum in the alloy would tend to introduce an excessive amount of aluminum into the resulting cast iron. Also tests have shown that aluminum contents over 6% are decreasingly effective and therefore uneconomical after exceeding 10%.

The silicon content of the alloy should be at

50 least twice that of the aluminum and at least 6% in order that the aluminum and silicon oxides formed will make a fusible slag which will sepa-

55 rate readily from the molten metal. Also it was found that if the silicon content was 10% or greater, the resulting alloy became extremely fri-

able. This is a very desirable feature in that it permits low cost crushing of the material which

55 will permit the production of the alloy at a lower cost than would be possible if shotting were nec-

essary. Also, many authorities are of the opinion that a crushed alloy is more desirable due to the

small sizes that may be available. The rate of

solution will therefore be more rapid since the

ratio of surface to mass is larger. The upper

limit of 25% silicon is based on the fact that a

higher percentage would introduce a detrimental

amount of silicon into the resulting cast iron.

The optimum percentage of silicon in the alloy is

between 10% and 15%.

The manganese content of the alloy can be

varied over a fairly wide range, though of course

manganese is not absolutely essential and there-

fore may be absent. It has a beneficial effect both

in increasing the effectiveness of the lower alum-

inum content alloy and also in lowering the final

cost of the alloy. Manganese is also very helpful in forming a low melting point slag which readily separates from the molten iron. It appears that a very low manganese alloy or even a manganese free alloy will have a considerable degree of the beneficial effects of these alloys. More than 25% manganese is not advisable because it would raise the final manganese content of the resulting cast iron excessively. Although an increase in the manganese content of the cast iron acts as a strengthener, the buyers of cast iron frequently set very definite limits on the manganese range. Any alloy which would tend to raise the manganese content to a marked degree, would, of course, increase the difficulty of maintaining a fixed manganese content in the cast iron. In some cases it would be necessary to keep the manganese content of the alloy to a minimum. The optimum amount of manganese in the alloy is believed to be approximately 10%, although up to 25% may be used.

The percentage of copper in the above alloy should be as high as possible due to its beneficial effect both as a strengthener and toughener of cast iron and also as regard its effect on reduction of chill and section sensitivity and on increasing the machinability. Copper provides, (1) a base to carry the "deoxidizing" element and the slag forming elements, (2) a means of introducing a large amount of alloy to the cast iron without causing foundry defects, and (3) introduces beneficial effects other than those obtained from the use of a "deoxidizer" alone.

The melting point of the above mentioned alloy is relatively low, being approximately 1500° F., though it varies somewhat over the composition range specified. This is an important point, because it permits fairly large additions of the alloy to be made to cast iron without materially lowering the metal temperature. It also tends to eliminate any tendency toward blowholes and other foundry defects that frequently accompany ladle additions of high melting point alloys. Even if comparable results could be obtained from the independent additions of aluminum, ferrosilicon, ferromanganese and copper to the ladle, the low melting point of the combined alloy would be an entirely justifiable reason for using it in preference to the separate components.

In the development of my invention, four different alloys were made in a small induction electric furnace lined with a clay graphite crucible. The melting practice was as follows: Ferrosilicon and ferromanganese were placed in the bottom of the furnace and covered with copper shot. When this charge was completely molten, the power was shut off, and aluminum was added in

the form of wire. The resulting alloy was poured into small dry sand pig molds. In every case the alloy was crushed to pass a 6 mesh screen and was retained on a 28-mesh screen. The alloys were designated as follows:

### Alloy 1:

|          | Percent |
|----------|---------|
| Aluminum | 3       |
| Silicon  | 9.5     |
| Iron     | 0.5     |
| Copper   | 87      |

### Alloy 2:

|           | Percent |
|-----------|---------|
| Aluminum  | 3       |
| Silicon   | 9.5     |
| Manganese | 10      |
| Iron      | 2.5     |
| Copper    | 75      |

## 20 Alloy 3:

|          | Percent |
|----------|---------|
| Aluminum | 6       |
| Silicon  | 12      |
| Iron     | 2       |
| Copper   | 80      |

### Alloy 4:

|           | Percent |
|-----------|---------|
| Aluminum  | 6       |
| Silicon   | 13      |
| Manganese | 10.5    |
| Iron      | 2.5     |
| Copper    | 68      |

35 Cast iron melts were made in an 120 lb. induction electric furnace lined with a magnesia crucible. The charge for each heat was essentially the same and consisted of pig iron, scrap steel, ferromanganese, ferrosulfide and ferro-silicon. The ferro alloys were added to the charge before melting was complete. Three 40 lb. ladles 40 were poured from each 120 lb. heat. Each ladle of iron was treated with the desired ladle addition as indicated in the following tables. The ladle addition was made to the stream of metal while 45 transferring the metal from the furnace to the ladle. The molten iron was allowed to cool to 2550° F. before pouring into green sand molds. Four 1.2 inch standard arbitration bars were contained in each mold. One mold was poured from 50 each ladle of iron.

50 The arbitration bars were tested for transverse strength, deflection, tensile strength and Brinell hardness according to standard procedure. The areas under the transverse strength-deflection 55 curves were used as a measure of resilience.

All values shown in the following tables are the average of four tests.

*Average physical properties of cast irons inoculated with ferrosilicon, copper and ferrosilicon, and aluminum-silicon-copper alloy 1*

| Bar No. | Max. temp. | Ladle addition | Trans. load | Trans. deflec-tion | Resili-ence | T. S.                 | Brinell hard-ness | T. C. | Si   | Cu    |
|---------|------------|----------------|-------------|--------------------|-------------|-----------------------|-------------------|-------|------|-------|
|         | °F.        |                | Pounds      | Inches             | In.·lbs.    | Lbs./in. <sup>2</sup> |                   | Pct.  | Pct. | Pct.  |
| 1.      | 2550       | .045# Fe Si    | 2450        | 0.285              | 440         | 32,500                | 180               | 3.32  | 1.92 | ----- |
| 2.      | 2550       | .045# Fe Si    | 2575        | 0.270              | 430         | 36,000                | 193               | 3.28  | 1.87 | .95   |
| 3.      | 2550       | .39% Cu        |             |                    |             |                       |                   |       |      |       |
| 4.      | 2750       | .45# alloy 1   | 2655        | 0.278              | 450         | 36,500                | 197               | 3.30  | 1.92 | .78   |
| 5.      | 2750       | .045# Fe Si    | 2350        | 0.232              | 340         | 32,000                | 186               | 3.25  | 1.86 | ----- |
| 6.      | 2750       | .045# Fe Si    | 2465        | 0.247              | 390         | 34,500                | 191               | 3.21  | 1.89 | .94   |
| 7.      | 2750       | .45# alloy 1   | 2555        | 0.261              | 435         | 38,500                | 207               | 3.17  | 1.83 | 1.02  |
| 8.      | 3000       | .045# Fe Si    | 2340        | 0.216              | 330         | 32,000                | 190               | 3.19  | 1.93 | ----- |
| 9.      | 3000       | .39% Cu        |             |                    |             |                       |                   |       |      |       |
| 8.      | 3000       | .045# Fe Si    | 2510        | 0.225              | 350         | 35,500                | 206               | 3.17  | 1.87 | .91   |
| 9.      | 3000       | .45# alloy 1   | 2615        | 0.234              | 380         | 40,500                | 210               | 3.15  | 1.89 | 1.09  |

*Average physical properties of cast irons inoculated with ferrosilicon, alloy 2 and alloy 3*

| Bar No. | Max. temp. | Ladle addition | Trans. load | Trans. deflec- | Resili-  | T. S.                 | Brinell hard- | T. C. | Si   | Cu    |
|---------|------------|----------------|-------------|----------------|----------|-----------------------|---------------|-------|------|-------|
|         | °F.        |                | Pounds      | Inches         | In.-lbs. | Lbs./in. <sup>2</sup> |               | Pct.  | Pct. | Pct.  |
| 10.     | 2550       | .045# Fe Si    | 2450        | 0.275          | 430      | 32,500                | 187           | 3.29  | 1.84 | ----- |
| 11.     | 2550       | .45# alloy 2   | 2620        | 0.278          | 460      | 38,500                | 200           | 3.28  | 1.83 | .76   |
| 12.     | 2550       | .45# alloy 3   | 2810        | 0.291          | 510      | 35,000                | 206           | 3.24  | 1.91 | 1.07  |
| 13.     | 2750       | .045# Fe Si    | 2320        | 0.240          | 360      | 33,000                | 191           | 3.31  | 1.86 | ----- |
| 14.     | 2750       | .45# alloy 2   | 2620        | 0.279          | 460      | 37,500                | 204           | 3.24  | 1.84 | .90   |
| 15.     | 2750       | .45# alloy 3   | 2670        | 0.292          | 490      | 38,000                | 205           | 3.24  | 1.86 | .88   |
| 16.     | 3000       | .045# Fe Si    | 2500        | 0.232          | 380      | 32,500                | 197           | 3.17  | 1.80 | ----- |
| 17.     | 3000       | .45# alloy 2   | 2610        | 0.242          | 430      | 39,500                | 214           | 3.16  | 1.80 | .91   |
| 18.     | 3000       | .45# alloy 3   | 2740        | 0.277          | 500      | 41,000                | 213           | 3.14  | 1.76 | .76   |

*Average physical properties of cast irons inoculated with ferrosilicon, alloy 3 and alloy 4*

| Bar No. | Max. temp. | Ladle addition | Trans. load | Trans. deflec- | Resili-  | T. S.                 | Brinell hard- | T. C. | Si   | Cu   |
|---------|------------|----------------|-------------|----------------|----------|-----------------------|---------------|-------|------|------|
|         | °F.        |                | Pounds      | Inches         | In.-lbs. | Lbs./in. <sup>2</sup> |               | Pct.  | Pct. | Pct. |
| 19.     | 2550       | .045# Fe Si    | 2480        | 0.308          | 520      | 34,500                | 181           | 3.25  | 1.94 | .02  |
| 20.     | 2550       | .45# alloy 3   | 2685        | 0.298          | 520      | 36,000                | 200           | 3.23  | 1.92 | .83  |
| 21.     | 2550       | .45# alloy 4   | 2620        | 0.272          | 460      | 38,000                | 205           | 3.23  | 1.94 | .77  |
| 22.     | 2750       | .045# Fe Si    | 2360        | 0.239          | 370      | 33,500                | 193           | 3.23  | 1.91 | .02  |
| 23.     | 2750       | .45# alloy 3   | 2720        | 0.292          | 500      | 38,000                | 202           | 3.22  | 1.84 | .84  |
| 24.     | 2750       | .45# alloy 4   | 2740        | 0.282          | 490      | 37,500                | 207           | 3.21  | 1.89 | .76  |
| 25.     | 3000       | .045# Fe Si    | 2365        | 0.242          | 370      | 35,500                | 189           | 3.22  | 2.03 | .02  |
| 26.     | 3000       | .45# alloy 3   | 2630        | 0.271          | 465      | 37,500                | 207           | 3.20  | 1.96 | .93  |
| 27.     | 3000       | .45# alloy 4   | 2600        | 0.264          | 440      | 37,000                | 207           | 3.22  | 1.94 | .65  |

*Average physical properties of cast irons inoculated with ferrosilicon and varying amounts of alloy 3*

| Bar No. | Max. temp. | Ladle addition | Trans. load | Trans. deflec- | Resili-  | T. S.                 | Brinell hard- | T. C. | Si   | Cu    |
|---------|------------|----------------|-------------|----------------|----------|-----------------------|---------------|-------|------|-------|
|         | °F.        |                | Pounds      | Inches         | In.-lbs. | Lbs./in. <sup>2</sup> |               | Pct.  | Pct. | Pct.  |
| 28.     | 3000       | None           | 2190        | 0.240          | 350      | 29,000                | 179           | 3.26  | 1.81 | ----- |
| 29.     | 3000       | .25# Fe Si     | 2420        | 0.334          | 540      | 30,500                | 170           | 3.21  | 2.32 | ----- |
| 30.     | 3000       | .45# alloy 3   | 2680        | 0.317          | 570      | 36,000                | 197           | 3.25  | 1.93 | .83   |
| 31.     | 3000       | None           | 2330        | 0.231          | 355      | 39,000                | 183           | 3.24  | 1.92 | ----- |
| 32.     | 3000       | .25# Fe Si     | 2280        | 0.331          | 500      | 30,500                | 167           | 3.17  | 2.49 | ----- |
| 33.     | 3000       | .60# alloy 3   | 2520        | 0.281          | 465      | 34,500                | 199           | 3.24  | 2.05 | .98   |
| 34.     | 3000       | None           | 2330        | 0.206          | 310      | 32,000                | 194           | 3.20  | 1.84 | ----- |
| 35.     | 3000       | .25# Fe Si     | 2250        | 0.322          | 490      | 32,000                | 172           | 3.18  | 2.37 | ----- |
| 36.     | 3000       | .80# alloy 3   | 2740        | 0.304          | 550      | 40,500                | 210           | 3.17  | 1.98 | 1.20  |

Based on the above data alone, it is obvious that the aluminum-silicon-copper alloys and the aluminum-silicon-manganese-copper alloys have a beneficial effect on cast iron. The increase in value for deflection shows that these alloys inhibit the formation of "dendritic" graphite in cast iron. It will also be apparent that these alloys do not introduce any weakening or detrimental elements such as are introduced by the addition of ferrosilicon in sufficient quantities to yield comparable "deoxidizing" effects, the degree of "deoxidizing" being indicated by the value for deflection, with low deflection usually indicating dendritic graphite.

That the "dendritic" graphite was inhibited by the use of my alloys was verified by examination of the fractures of the bars which were a clean bright gray characteristic of normal cast iron, instead of being dark and sooty as characteristic of "modified" cast iron.

Due to the low melting point of my alloys, no difficulty was encountered in adding them to molten cast iron, even to small ladles at low temperatures. The optimum or economical amount of these alloys to be added appears to be 1%. The best of those alloys studied were those containing 6% aluminum.

In view of the above and other published and unpublished information concerning the phenomenon of modified cast iron, it is believed that my alloys serve as a deoxidizing agent for cast iron

45 which is superior to previously known "deoxidizing" agents and which impart to the cast iron benefits other than those due to "deoxidizing" alone. It is low in cost and is easily added to and readily absorbed by the molten cast iron without introducing any weakening or detrimental effects or foundry defects such as blow holes and excessive shrinkage. When added in proper percentages, it improves the physical and mechanical properties of the cast iron.

55 Having thus described my invention, what I claim is:

1. A method of making gray cast iron which consists in adding to the cast iron when it is in a molten state a copper base alloy in effective amounts up to 2 per cent of the total melt, said copper base alloy consisting of 1 to 10 per cent aluminum, 6 to 25 per cent silicon, manganese in effective amounts up to 25 per cent and copper in excess of 50 per cent, the balance being substantially all iron but not exceeding 30 per cent.

2. A material for addition to molten iron, which will be gray iron when cast, for the purpose of inhibiting or decreasing modification of the cast iron comprising a copper base alloy consisting of 1 to 10 per cent aluminum, 6 to 25 per cent silicon, manganese in effective amounts up to 25 per cent and copper in excess of 50 per cent, the balance being substantially all iron but not exceeding 30 per cent.

THOMAS E. BARLOW.